

March 1, 1938.

K. FUJII ET AL.

2,109,839

PROCESS FOR MANUFACTURING METAL COATED THREAD

Filed Dec. 9, 1933



INVENTORS:  
Kitaro Fujii, and  
Seiichiro Iwamoto.  
BY Baseltine, Lake & Co.  
ATTORNEYS.

## UNITED STATES PATENT OFFICE

2,109,839

## PROCESS FOR MANUFACTURING METAL COATED THREAD

Kitaro Fujii, Otomura, Nakakouchi-gun, Prefecture Osaka, and Seiichiro Iwamoto, Osaka, Japan

Application December 9, 1933, Serial No. 701,722  
In Japan December 19, 1932

2 Claims. (Cl. 91—68)

This invention relates to a process for manufacturing metal coated thread, and its object is to produce easily and economically a metal coated thread of greater strength and higher luster than that made by usual processes, with least possibility of the metal peeling off.

Metal coated thread has heretofore been manufactured by drawing a thread, on which paste has been applied, through metallic dust. The thread thus manufactured lacks sufficient lustre, smooth surface, and is not perfectly round. Also the metallic powder comes off easily, and is not satisfactory in practical use.

In accordance with this invention, we have made use of small pieces of metal leaf instead of metallic powder, and put them into a solution of paste. The metal leaves, in suspension in the solution of paste, are put on a core thread by drawing the thread through a special capillary tube. Such capillary tube is put on or forms the tip of a gradually converging nozzle and has the diameter corresponding to the finished thread before the paste has become dry, thereby obviating the above mentioned defects, and providing excellent metal coated thread.

This we consider to be novel, and our invention will be better understood by reference to the following specification and appended claims when considered in connection with the accompanying drawing.

Fig. 1 is an enlarged sectional view of a capillary nozzle having gradually converging diameter for carrying this invention into effect; Figs. 2 and 3 are enlarged sectional views showing expandable capillary nozzle tips.

Referring to Fig. 1 of the drawing, 1 represents a capillary tube fitted to the tip end of a capillary nozzle 5 which is supplied with the solution of paste 2 with the thin metallic leaves 3 in suspension. The thread 4 is drawn through the gradually converging nozzle and capillary tube. Then the thread comes out of the capillary tube with a uniform coating of small leaves of metal foil.

Thread is not generally uniform in diameter, having lumps and joints, in which case the capillary tubes as shown in Figs. 2 and 3 are preferably used. The capillary tubes as shown in Figs. 2 and 3 are made of flexible tubular metal plate, having overlapping portions 6 and 7 which are self-adjusting. Under normal conditions, the capillary tube keeps its smallest diameter, but when a lump 8 passes through the tube, it expands automatically, as shown in Fig. 3 to ac-

commodate the irregularities, thereby preventing the breaking of the thread.

For this purpose, a capillary tube, consisting of two or more separate pieces, joined together to accommodate irregularities in the diameter, may equally be used.

In another way of carrying this invention into effect, the same object can be attained by passing the thread through the solution of paste having the metal leaves in suspension. The thread thus coated with the metallic leaves is drawn through the capillary nozzle having a gradually converging circular hole.

Now we will explain an actual example more in detail.

The mixed solution of 3.37% of cotton nitrate; 16.74% of butyl acetate; 13.95% of acetone; 27.97% of benzene; 4.46% of ester gum; 28.57% of butylphthalate is mixed with six parts of liquid consisting of 4 parts of benzene and 6 parts of ether to obtain a viscous paste. This paste is put in a container provided with a capillary nozzle 1 at its one extremity as shown in Fig. 1. Small pieces of metal leaf 3, smaller than 50 mesh, of an alloy consisting of copper, tin, zinc and iron, having specific gravity of 7.93, are put into the paste 2. The thread 4 is passed through the paste in the direction of the arrow a at the speed of 20 centimeters per second. The metallic leaves 3 suspended in the paste will be subject to the force as shown by arrows b due to the forward movement of the thread 4, which will bring the leaves floating at random in the broader part of the convergent nozzle, in positions parallel with the surface of the thread in the tip of capillary tube 1. When the thread is drawn thru the capillary tube, the flat leaves are pressed firmly on to the thread surface and attached thereto as if they were wound. Metal coated thread thus manufactured has high lustre and durability against abrasion. It also has other useful characteristics such as strong tensile strength and uniformity of diameter and finish.

All metals generally consist of an aggregation of fine crystals, each arranged irregularly in indefinite directions, therefore the powder obtained by crushing such metal gives diffused reflections on the surface, and has unsatisfactory lustre. On the other hand it has been found by X-ray analysis, that small pieces of thin metal leaf obtained by cold press work has a fibrous texture in which the crystals are arranged in parallel with the flat surface of the leaf giving better luster on the surface than on the section. In this invention we have made use of the thin metal

leaf as the necessary condition for improving metal coated thread.

Since thread generally consists of an assembly of a number of single fibres twisted together, there are many spaces and irregularities in it. In order to increase the strength of the metal covered thread and the durability of the metal covering, it is necessary to utilize the above mentioned spaces for containing as much paste as possible, and pressing the metal leaves very firmly thereon.

As above described, in accordance with this invention, a capillary nozzle is used which has a gradually converging inner diameter, while the nozzle tip has a diameter almost equal to that of a finished thread. When the thread is to be coated, the leaves are firmly pressed onto the surface of the thread, guided by the inner wall of the gradually convergent capillary nozzle while passing therethrough.

20 The metal coated thread manufactured by the method of the present invention has such construction that the flat surface of each thin metal leaf is firmly pressed onto the surface of the core thread in parallel thereto, causing a very desirable lustre, owing to the special shine inherent to the flat leaves, and uniform reflection of light. Moreover since the paste penetrates into the thread filling the spaces and irregularities, it has greater strength than ordinary golden or silver threads manufactured by former processes. The paste prevents the metal leaves from becoming 25 rusty.

What we claim as new and desire to secure by Letters Patent of the United States is:

35 1. The method of manufacturing metallic threads, such as golden or silver threads, which consists in drawing a core thread through a paste solution which contains a quantity of very small

flat metal flakes in suspension and finally pulling out said thread through a capillary nozzle having a gradually converging orifice and having a nozzle tip of an interior diameter almost equal to that of a thread to be finished, said capillary nozzle and nozzle tip being filled with the paste solution containing said metal flakes in suspension and said gradually convergent nozzle acting to collect the metal flakes towards the nozzle tip by the movement of the core thread therethrough so as to cause the metal flakes to be deposited and accumulated uniformly and evenly around the thread and firmly pressed together to incorporate with the surface of said thread in passing through the nozzle tip.

2. The method of manufacturing metallic threads, such as golden or silver threads, which consists in drawing a core thread through a paste solution which contains a quantity of very small flat metal flakes in suspension and finally pulling out said thread through a capillary nozzle having a gradually converging orifice and having a resiliently expandible nozzle tip of an interior diameter almost equal to that of a thread to be finished and capable of expanding to allow for inequalities in the thread, said capillary nozzle and nozzle tip being filled with the paste solution containing said metal flakes in suspension and said gradually convergent nozzle acting to collect the metal flakes towards the nozzle tip by the movement of the core thread therethrough so as to cause the metal flakes to be deposited and accumulated uniformly and evenly around the thread and firmly pressed together to incorporate with the surface of said thread in passing through the nozzle tip.

KITARO FUJII.  
SEIICHIRO IWAMOTO.